

Aug. 9, 1949.

G. CROYERE  
PLASTIC BITUMINOUS MATERIAL AND  
METHOD OF MAKING THE SAME  
Filed April 9, 1946

2,478,654

*Fig. 1.*



*Fig. 2.*



INVENTOR.

*G. Croyere*

BY

*Gloucester Downing Peckle  
Attorneys.*

## UNITED STATES PATENT OFFICE

2,478,654

PLASTIC BITUMINOUS MATERIAL AND  
METHOD OF MAKING THE SAMEGhislain Croyere, Decazeville, France, assignor to  
Louvreil-Montbard-Aulnoye, Paris, France, a  
body corporate of FranceApplication April 9, 1946, Serial No. 660,624  
In France October 27, 1944Section 1, Public Law 690, August 3, 1946  
Patent expires October 27, 1964

4 Claims. (Cl. 196—74)

1

Coal tar pitch as obtained by the distillation of the tar from coke plants, town-gas plants, gas producers, etc., is frequently used for the production of water-tight linings on roofs, terraces, metal parts to be buried or immersed, etc.

In most of such applications the said pitch suffers from the major inconvenience that it is exceedingly sensitive to variations in temperature. While being very brittle in the cold, it will soften as soon as temperature rises somewhat. Moreover, it is subject to flow considerably, that is, it will undergo deformation by the effect of its own weight whenever it is laid in a layer of substantial thickness sloping towards the horizontal. This phenomenon is particularly evident at those temperatures at which the product is comparatively soft, although it is still very appreciable at temperatures at which pitch has taken a hard and brittle character. Last, pitch is subject to the phenomenon known as "aging." A layer of pitch when left exposed to the action of the air will crack rapidly. Such cracks frequently reach a considerable depth and thus impair the water-tightness of the lining. The pitch assumes an increasingly hard and brittle character and the structure is infallibly doomed to destruction unless the aging of the lining is cured in time.

These peculiarities considerably restrict the field of application of pitch inasmuch as they involve among others the following inconveniences:

1. The linings will crack by the action of cold (which seems to be due to the fact that pitch becomes very brittle in the cold and thus can no longer resist the stresses due to shrinkage);

2. Sloping linings cannot be laid in rather thick layers because the pitch would flow, that is, would creep down the lined surface;

3. Metal parts to be buried, such as metal tubes, etc., are most insufficiently protected, since the coatings will not stand the handling of said parts, or will be chipped off by even the slightest knock, or will be squeezed away by the weight of the part if the latter is exposed to the sun, etc.

4. Aging will make the protection most uncertain after a generally short time.

Attempts have been made partly to remedy the said inconveniences by admixing pitch with various coal tar oils ("fluxing") or mineral or some other fillers in dust form ("filling"), pebble (pitch concrete), cardboard, felt, fabric, etc. Frequently, several of these expedients are used together. Except those materials which are obtained by the association of straight or "filled"

2

or "fluxed" pitch with fabrics, cardboard, felt and the like, the chief effect of the addition of fluxes or fillers to pitch is to modify the properties of the latter with a view to adapt them to the required conditions of use, but it has no decisive effect upon the properties discussed above, viz.: temperature sensitiveness, aging, flowing.

Similar properties are found although to a much less degree in pitch manufacture notably by oxidation from mineral oils, so that same generally is preferred to coal tar pitch for waterproofing and anticorrosive purposes. However, the cost of such products is much higher.

Now applicant has found that it is possible to correct in a very efficient manner the above mentioned drawbacks in the case of coal tar pitch by means of a very simple industrial method so as to obtain reconstituted or reformed pitches, the properties of which approximate very closely those of mineral oil pitches while their cost price is much less than that of said mineral oil pitches and the said improved reconstituted pitches may be advantageously applied in a large number of cases and more particularly for fluid-tight structures.

It has already been proposed to incorporate anthracene paste to coal-tar pitch, said anthracene paste being the solid product separating after cooling from certain oils obtained through distillation of coal tar or tar obtained in gas plants, coke plants or gas producers. But such anthracene paste was used heretofore only as a flux, that is with a view to obtaining a lowering of the softening point of the original pitch. Such prior mixtures serve in particular for the production of fuel agglomerates such as coal dust or brown coal dust briquettes and the like.

However, the applicant has found that the properties of pitch-anthracene paste mixtures undergo unexpected but highly valuable alterations depending on the respective percentages of pitch and anthracene paste.

The invention is illustrated in the accompanying drawings in which

Fig. 1 is a diagrammatic view illustrating the general course of the melting curve, the percentages of anthracene and the melting points of the mixture, and

Fig. 2 is a ternary diagram with the curve defining the proportions between the pitch anthracene and the coal tar oil.

In particular if the softening point of a mixture of coal tar pitch and anthracene paste is defined for instance with the ring and ball method

of the American Society for Testing Material, it is found that said point of softening first decreases down to an approximative content of 15% of anthracene paste. It then rises suddenly until said content reaches a value comprised between 30 and 40% and it varies subsequently only in a very slow manner (see Fig. 1). It is apparent that the constitution of the mixture is clearly different according to the proportions to be foreseen for the two components by reason of the modifications mentioned hereinabove as concerns the physical and mechanical properties of the mixture which properties are entirely different to either side of the point marked B in Fig. 1. But the point that should be primarily remarked consists in that a little before the point marked C on the curve, that is the point beyond which the variations in the softening temperature becomes very slow, the mixture obtained shows properties approximating closely those of mineral oil pitches.

The applicant has also found that a new physical constituent will result from an infinity of proportions between pitch, anthracene and coal tar oil that are defined by curve abc of the ternary diagram shown in Fig. 2. In the said diagram apex I represents a highly dry pitch (with a K.S. melting point higher than 100° C.), II represents an ordinary anthracene oil and III the crystal mass separated as explained above, then carefully drained and finally stripped of every trace of mother oil by extraction with a suitable solvent such as ethyl alcohol. Points on curve abc indicate the melting temperatures of the corresponding mixtures.

The following examples are illustrative of the properties that can be obtained by the method described hereinbefore.

The following materials are used:

|                                                                                                                                                                   | Per cent |
|-------------------------------------------------------------------------------------------------------------------------------------------------------------------|----------|
| Coke plant tar pitch M. P. (K. S.) 70° C.                                                                                                                         | 65.5     |
| Raw drained commercial anthracene from the fraction 290-380° C., containing 32% of ethanol-soluble oils and melting between 110 and 130° C. in the de-oiled state | 34.5     |

The mixture is melted. The product obtained possesses the following properties:

|                                        |        |
|----------------------------------------|--------|
| M. P. (K. S.)                          | 80° C. |
| Penetration ASTM under 100 g. load at— |        |
| 25° C.                                 | 25     |
| 45° C.                                 | 185    |

Flowing: Completely null up to 65° C. Slight between 65 and 70° C.

Aging: With the above product aging makes itself noticeable by the formation of shallow and consequently wholly harmless wrinkles, even after three years exposure to the sun and inclemencies.

A better appreciation of the importance of this invention will be had from the following statement, given by way of example, of the characteristics of a good fluxed coal tar pitch and a mineral oil pitch which are similar as to the results of the penetration test at 25° C.

#### 1.—Coal tar pitch

|                                    |                             |
|------------------------------------|-----------------------------|
| M. P. (K. S.)                      | 55° C.                      |
| ASTM penetration test (100 g.) at— |                             |
| 25° C.                             | 25                          |
| 45° C.                             | Too large to be measurable. |

Flowing: The pitch has flowed completely at 25° C. It even flows at 0° C.

Aging: Deep cracks reaching the whole thickness of the pitch layer after exposure of the same.

Moreover, the applicant has found that the product obtained in the performance of this method can be improved considerably by physical treatments to be carried out upon either the product itself or the raw materials involved in the production thereof.

The said physical treatments are those which are usually employed for resinifying the oily and low-boiling constituents of pitch and generally of coal tar derivatives. Such are:

1. Oxidation by air-blowing,
2. Chlorination with the aid of a mixture of chlorine with air or of chlorine alone,
3. Sulfuration by means of sulphur or other derivatives belonging to the chemical family of sulfur,

4. Polymerization with the aid of metal salts such as iron perchloride, aluminum chloride or other salts,

5. Co-polymerization by means of synthetic resins whose molecules are capable of providing linkages between the molecules of the oils present, such as resins belonging to the vinyl, or the acryl, or the methacryl, or the styrene series.

Briefly stated, every substance capable of fixing in larger molecular structures those too low-boiling compounds whose escape is one of the main causes of aging can be used.

The applicant does not intend to protect the application of the above-enumerated treatments to every coal tar oil and pitch but only to the above-described product and to the raw materials involved in the production thereof.

The examples given hereinafter are illustrative of the properties that can be obtained by resinification of pitch-oil-anthracene mixtures defined in the above. For the sake of simplicity the said mixture will be referred to as "product No. 1."

*Example 1.*—Blowing product No. 1 by means of an air stream passed through the molten mass at the rate of half a liter per kilogram of material and per minute.

Temperature of the melt: 190° C. Duration: 4 hours.

*Example 2.*—Admixing product No. 1 with 10% by weight of anthracene oil and blowing the mixture with a mixture of air with 5% by volume of chlorine fed at the rate of half a liter per kilogram of material and per minute.

Temperature of the melt: 190° C. Duration: 4 hours.

*Example 3.*—Treating product No. 1 for 3 hours at a temperature of 220° C. with  $\frac{1}{20}$  of its own weight of sulfur flour.

*Example 4.*—Admixing product No. 1 with 2% by weight of anhydrous iron chloride and heating the mixture for 3 hours at 250° C.

*Example 5.*—Admixing product No. 1 with 2% by weight of polyvinyl chloride and heating the mixture for 2 hours at 130° C.

*Example 6.*—Admixing product No. 1 with 5% of polyvinyl chloride and heating the mixture for 2 hours at 130° C.

65 The treatments defined by the above examples are effective to increase the stability of the product and to counteract aging.

What I claim as my invention and desire to secure by Letters Patent is:

1. A plastic bitumen-like material of very low temperature sensitivity and flow capacity constituted by a mixture of about 65% of coal tar pitch with about 35% by weight of commercial anthracene paste.

70 2. A method for producing a bitumen-like ma-

material having a very low flow capacity and temperature sensitivity, consisting in melting and mixing together about 65 parts of coal tar pitch by weight with about 35 parts by weight of raw commercial anthracene paste.

3. A method for producing a bitumen-like material having a very low flow capacity and temperature sensitivity, consisting in melting and mixing together about 65 parts of coal tar pitch by weight with about 35 parts by weight of raw commercial anthracene paste and incorporating to the mixture a filler substance.

4. A method for producing a bitumen-like material having a very low flow capacity and temperature sensitivity, consisting in melting and mixing together about 65 parts of coal tar pitch by weight with about 35 parts by weight of raw commercial anthracene paste and oxidizing the molten mixture through blowing.

GHISLAIN CROYERE. 20

#### REFERENCES CITED

The following references are of record in the file of this patent:

#### UNITED STATES PATENTS

| Number      | Name             | Date           |
|-------------|------------------|----------------|
| 924,086     | Meadows et al.   | June 8, 1909   |
| 1,266,261   | Henderson        | May 14, 1918   |
| 5 2,059,051 | Sparks           | Oct. 27, 1936  |
| 2,093,450   | Jacobsohn        | Sept. 21, 1937 |
| 2,095,190   | Heuscher         | Oct. 5, 1937   |
| 2,220,714   | Hersberger       | Nov. 5, 1940   |
| 2,281,728   | Thelen           | May 5, 1942    |
| 2,287,511   | Burk et al.      | June 23, 1942  |
| 2,297,455   | Brautigam et al. | Sept. 29, 1942 |
| 2,348,832   | Mauch et al.     | May 16, 1944   |
| 2,395,853   | Fair             | Mar. 5, 1946   |

#### FOREIGN PATENTS

| Number  | Country             | Date          |
|---------|---------------------|---------------|
| 1,428   | Great Britain, 1914 | Apr. 19, 1915 |
| 216,245 | Great Britain       | May 29, 1924  |
| 216,602 | Great Britain       | June 5, 1924  |

#### OTHER REFERENCES

Abraham, "Asphalts and Allied Substances," 4th Edition, pages 366 and 367, published by D. Van Nostrand Co.